

Nov. 17, 1925.

1,562,383

C. M. TAYLOR

FLOOR COVERING AND PROCESS OF MAKING SAME

Original Filed Jan. 10, 1922

*FIG. 1.*



*FIG. 2.*



Inventor

*C. Marshall Taylor*

By *Prentiss, Stone & Boyden*  
Attorneys.

## UNITED STATES PATENT OFFICE.

CALEB MARSHALL TAYLOR, OF ELIZABETH, NEW JERSEY.

## FLOOR COVERING AND PROCESS OF MAKING SAME.

Application filed January 10, 1922, Serial No. 528,298. Renewed September 1, 1925.

*To all whom it may concern:*

Be it known that I, CALEB MARSHALL TAYLOR, a citizen of the United States, residing at Elizabeth, in the county of Union 5 and State of New Jersey, have invented certain new and useful Improvements in Floor Coverings and Processes of Making Same, of which the following is a specification.

This invention relates to floor coverings 10 and to a process of making the same.

The floor covering provided is of that type known as felt base floor coverings and particularly such materials in which an asphalt or bitumen impregnated base is used.

15 The invention is also peculiarly adapted for use in combination with all floor coverings in which either the wear surface or the opposite face is formed of paint or other material containing linseed oil or other oil, 20 or any material subject to saponification, or removable under the action of soap and the usual floor cleaning materials.

25 Bitumen impregnated felt base floor coverings may be recognized by the main dark body which is particularly evident when the material is cut. The felt of such bases may be made from rags, or from paper or any cellulose material, or from a mixture of such materials, thoroughly impregnated 30 with asphalt or tar or some suitable bituminous material. When used as a supporting base for floor covering it is the usual practice to coat the bitumen impregnated base with a layer of paint which is known as the 35 sealing coat and often to apply various painted designs, all of which may be applied in any convenient manner. Also, a coat of paint is applied to the opposite or under surface of the impregnated base to cover the dark and unsightly bitumen impregnated base.

40 For the manufacture of such bitumen impregnated bases it has been found that the wear paint and the decorative paint may become discolored due in part to the inherent 45 nature of the bitumen of the base. Also in drying the paint coats it is necessary to dry at relatively low temperatures and for a longer period of time, often as long as four 50 or five days. A higher temperature and more rapid drying would tend to liquefy the bitumen and delay proper drying of the paint and also discolors the paint due to the release of materials from the base. Thus 55 a baking temperature of 175° F. or more,

such as is desirable for treating the paint coats, is not advisable in the usual drying of such coated bases.

After the present known product is completed it is usually necessary to place paper 60 between adjacent surfaces when the material is rolled or stacked in layers to prevent the adjacent painted surfaces from adhering. It is well known that all such painted surfaces, and also that the surface of the material known as linoleum, are worn away by the use of soap and water because of saponification by such cleaning materials on the oils in the paint and linoleum.

65 The present invention provides a coating 70 of a non-saponifiable material on one or both faces of the bitumen impregnated floor covering base. If the sides or marginal edges are also covered, the covering constitutes a sealing coating peculiarly adapted 75 for use on rug sizes of floor coverings. Thus the relatively inexpensive bitumen impregnated base may be used, the desirable features retained, and most of the undesirable characteristics eliminated. The paint coats 80 applied over the sealing coat do not become discolored by the material within the bitumen impregnated felt even when subjected to a baking temperature, and the time required for drying the paint coats is reduced 85 to a much shorter length of time than heretofore possible where similar impregnated bases are used.

90 In producing the floor covering of this invention, the usual asphalt or bitumen impregnated felt base is used. A solution is prepared of a mixture of nitrocellulose and a solvent therefor. Preferably the desired quantity of a semi-drying or drying vegetable oil is added to the mixture as a softening medium. It is desirable to add a quantity of resin. The solution is applied to one or both sides of the impregnated base as a sealing coat by any well known coating process. The solution thus applied is quickly dried on the base at a suitable drying temperature of approximately 140° F. The 95 impregnated base is thus provided with an impervious film which may be used wherever an ordinary bitumen impregnated base would before not have been acceptable on account of the sticky tarry nature of its materials. The coated base may be used as such for a floor covering or preferably may be further coated with wear and decorative 100 105 110

paint coats, or the sealing pyroxylin coat may carry a pigment to give the desired shade of color.

Other cellulose esters than nitrocellulose, such as acetyl cellulose, may be used.

One satisfactory mixture for the coating solution may be made by using 12 parts by weight of nitro cotton, and 88 parts by weight of a solvent mixture which may be composed of 35 per cent of acetone oil and 65 per cent of such a diluent as solvent naphtha, xylol, toluol, or benzol. Any well known working formula may be used for combining such a mixture of drying or semi-drying vegetable oil and nitro cotton. To such a mixture 12 parts by weight of linseed oil or other semi-drying or drying vegetable oil can be added. 12 parts of a resin, such as cumaron, may be added to advantage.

In the accompanying drawing, Figure 1 represents an enlarged sectional view of a sheet of impregnated felt base 1 having coatings of pyroxylin on the opposite faces thereof, indicated by 2 on the lower coat, and by 3 on the upper coat.

Figure 2 is a plan view of the material illustrated in Figure 1.

The sealing coat increases the tensile strength of the bitumen saturated base about 10 per cent. The sealing coat may advantageously be applied to the impregnated felt base at the felt impregnating factory and before shipment. The material possesses good wearing qualities whether it is considered as an underneath coating or as an upper wear coat.

The sealing coat on the back would prevent discoloring of the faces when the finished goods are rolled up or come in contact with each other.

I claim:

1. A floor covering comprising an asphalt impregnated felt base enclosed in a coating of a cellulose ester.
2. A floor covering comprising a bitumen impregnated felt base coated with a non-saponifiable film of cellulose ester.
3. A floor covering comprising a bitumen impregnated felt base having the opposite faces thereof coated with a sealing coat of a non-saponifiable film of cellulose ester.
4. A floor covering comprising a bitumen impregnated felt base having the opposite faces thereof coated with a film of a cellulose ester.
5. A floor covering comprising a bitumen impregnated felt base having the opposite faces thereof coated with a mixture of a cellulose ester and a softening medium.
6. A floor covering comprising a bitumen impregnated felt base having the opposite faces thereof coated with a mixture of a cellulose ester and a resin.
7. A floor covering comprising a bitumen impregnated felt base having the opposite

faces thereof coated with a mixture of a cellulose ester, a resin, and a vegetable oil.

8. A floor covering comprising a bitumen impregnated felt base coated with a mixture of a cellulose ester and resin.

9. A floor covering comprising a bitumen impregnated felt base coated with a mixture of a cellulose ester, a resin, and a vegetable oil.

10. A floor covering comprising an asphalt impregnated felt base enclosed in a coating of nitrocellulose.

11. A floor covering comprising a bitumen impregnated felt base coated with a film of nitrocellulose.

12. A floor covering comprising a bitumen impregnated felt base having the opposite faces thereof coated with a sealing coat of nitrocellulose film.

13. A floor covering comprising a bitumen impregnated felt base having the opposite faces thereof coated with a mixture of a nitrocellulose film and a softening medium.

14. A floor covering comprising a bitumen impregnated base coated with a film of a cellulose ester.

15. A floor covering comprising a bitumen impregnated base completely coated with a sealing coat of a nitrocellulose material.

16. The process of making floor coverings which comprises coating a bitumen impregnated felt base with a mixture of a solution of a cellulose ester, a resin, and a drying oil.

17. The process of making floor coverings which comprises coating a bitumen impregnated felt base with a solution of a cellulose ester, and drying the material thus prepared.

18. The process of making floor coverings which comprises coating a bitumen impregnated felt base with a mixture of a solution of a cellulose ester and a softening medium, and drying the material thus prepared.

19. The process of making floor coverings which comprises coating a bitumen impregnated felt base with a pigment colored solution of nitrocellulose.

20. The process of making floor coverings which comprises coating a bitumen impregnated felt base with a mixture of a solution of nitrocellulose and a softening medium.

21. The process of making floor coverings which comprises coating a bitumen impregnated felt base with a solution of nitrocellulose, and drying the material thus prepared.

22. The process of making floor coverings which comprises coating a bitumen impregnated felt base with a mixture of a solution of nitrocellulose and a softening medium, and drying the material thus prepared.

23. The process of making floor coverings which comprises coating a bitumen impregnated felt base with a solution of a cellulose ester, which solution contains approximately

- 12 parts by weight of a cellulose ester and 88 parts of solvent therefor.
24. The process of making floor coverings which comprises coating a bitumen impregnated felt base with a solution of a cellulose ester, which solution contains approximately 12 parts by weight of a cellulose ester, 88 parts of solvent therefor, and 12 parts of a softening medium.
- 10 25. The process of making floor coverings which comprises coating a bitumen impregnated felt base with a solution of nitrocellulose, which solution contains approximately 12 parts by weight of nitrocellulose and 88 parts of solvent therefor.
- 15 26. The process of making floor coverings which comprises coating a bitumen impregnated felt base with a solution of nitrocellulose, which solution contains approximately 12 parts by weight of nitrocellulose, 88 parts of solvent therefor, and 12 parts of a softening medium.
- 20 27. The process of making floor coverings which comprises coating a bitumen impregnated felt base with a solution of nitrocellulose, which solution contains a mixture of approximately 12 parts by weight of nitrocellulose, 88 parts of a solvent therefor, and 12 parts of a resin.
- 25 28. The process of making floor coverings which comprises coating a bitumen impregnated felt base with a solution of nitrocellulose, which solution contains a mixture of approximately 12 parts by weight of nitrocellulose, 88 parts of a solvent therefor, 12 parts of a resin, and 12 parts of a vegetable oil.
- 30 29. The process of making floor coverings which comprises coating a felt base impregnated with water resistant material with a solution of nitrocellulose, which solution contains a mixture of approximately 12 parts by weight of nitrocellulose, 88 parts of a solvent therefor, and 12 parts of a resin.
- 35 30. The process of making floor coverings which comprises coating a felt base impregnated with water resistant material with a solution of nitrocellulose, which solution contains a mixture of approximately 12 parts by weight of nitrocellulose, 88 parts of a solvent therefor, 12 parts of a resin, and 12 parts of a vegetable oil.
31. A smooth surface floor covering comprising an asphalt impregnated porous base enclosed in a coating of a film of a cellulose ester material.
- 35 32. A smooth surface floor covering comprising a porous fibrous base impregnated with bitumen and having the opposite faces thereof coated with a film of a cellulose ester material.

In testimony whereof I affix my signature.

CALEB MARSHALL TAYLOR.